

## UNITED STATES PATENT OFFICE

EMIL FENDT AND KARL SCHÖRG, OF FRANKFORT-ON-THE-MAIN-HOCHST, GERMANY,  
ASSIGNORS TO I. G. FARBEINDUSTRIE AKTIENGESELLSCHAFT, OF FRANKFORT-  
ON-THE-MAIN, GERMANY

## ELECTRICAL INDUCTIVE AND RESISTANCE HEATING DEVICE

No Drawing. Application filed December 19, 1928, Serial No. 415,346, and in Germany December 28, 1928.

The present invention relates to a heat-resisting electrical coil and to electrical resistance heating devices.

The windings of electrical induction apparatus are in some cases liable to be exposed to a temperature which is so high that normal insulating materials, such as cotton, paper or the like cannot be used. The wires have therefore been taped with asbestos which, however, at high temperatures, at about 300° C. loses its mechanical strength and begins to disintegrate. It has been tried to prevent this by impregnating the asbestos band with water glass, but this means also failed at temperatures of about 450° C. because the insulation was apt to fuse, causing a short-circuit.

According to this invention temperatures of about 750° C. can be attained in electrical resistance windings, as well as in induction coils, without causing a loss in mechanical and electrical strength of the insulation by impregnating the winding, which has been insulated with asbestos or a similar fibrous material, with a cement-mass substantially consisting of an acid-proof cementitious powder and containing one or more silicofluorides, preferably sodium silicofluoride in a quantity preferably ranging between about 3 and 10 per cent by weight. The mode of impregnation must be such that the wire to be insulated is during the winding everywhere well coated with the cement-mass. The several turns of the winding should be at 35 a distance of about 2 mm. from each other and the space between them should be filled with the cement-mass. The finished coil is caused to harden for some hours at a normal temperature (about 20° C. to 30° C.); it is then dried for some time, depending upon the thickness, at about 200° C. until the water is completely expelled. In case the coil has to be used at temperatures above 400° C. it has been found suitable to boil it, after it 45 has been hardened for about 20 hours, in

ordinary water in order to remove the residues of alkali and then to dry it.

When applying the present invention to electrical resistance heating devices, the object to be heated or parts thereof are covered with a moderately thick layer of the aforesaid cement-mass and on this layer one or several layers of asbestos millboard, asbestos band or similar fibrous material, likewise covered with the cement-mass, are wound. The 55 cement-mass is again applied to this insulating layer, and the resistance winding is placed upon the layer while the latter is still moist. The finished winding is then covered with a layer of asbestos which has been likewise 60 impregnated with the cement-mass.

In making heating plates in particular, the resistance winding is often directly pressed into the clayey mass. Cement-masses containing silicofluorides are also very suitable for this kind of construction. The 65 resistance material is introduced into the cement-mass which has been stirred to a paste. The further treatment is as described above.

We claim:

1. A heat-resisting electrical coil consisting of a layer of an insulating fibrous material, said insulating layer being impregnated with a cementitious substance containing a silicofluoride and an electrical conductor embedded in said layer. 70

2. A heat-resisting electrical coil consisting of a layer of asbestos, said layer being impregnated with a cementitious substance containing a silicofluoride and an electrical conductor embedded in said layer. 80

3. An electrical resistance heating device comprising a body to be heated, a layer of insulating cementitious material surrounding at least part of said body and a resistance coil of an electrically conductive material, embedded in said insulating cementitious material, said insulating cementitious material being characterized by the presence of 85 a silicofluoride therein. 90

4. An electrical resistance heating device comprising a body to be heated, a layer of insulating cementitious material surrounding at least part of said body, and a resistance coil consisting of an electrically conductive material and a layer of insulating fibrous material surrounding said conductive material, said insulating material and said cementitious material being characterized by the presence of a siliconfluoride therein.

10 In testimony whereof, we affix our signatures.

**EMIL FENDT.**  
**KARL SCHÖRG.**

**15**

**20**

**25**

**30**

**35**

**40**

**45**

**50**

**55**

**60**

**65**